

Nov. 10, 1953

E. F. PEVERE ET AL

**2,658,861**

## PROCESS FOR THE HYDROGENATION OF COAL

Filed Nov. 19, 1948



INVENTORS  
ERNEST F. PEVERE  
HOWARD V. HESS  
GEORGE B. ARNOLD

Daniel Shryer  
J. H. Graham  
ATTORNEYS

## UNITED STATES PATENT OFFICE

2,658,861

PROCESS FOR THE HYDROGENATION  
OF COAL

Ernest F. Pevere and Howard V. Hess, Beacon,  
and George B. Arnold, Glenham, N. Y., as-  
signors to The Texas Company, New York, N. Y.,  
a corporation of Delaware

Application November 19, 1948, Serial No. 61,012

2 Claims. (Cl. 196—62)

1

This invention relates to a process for the hydrogenation of coal. The process of this invention is particularly applicable to the treatment of bituminous coals.

In the conventional coal hydrogenation processes, such as practiced in Germany, the coal is dried, pulverized, and made into a paste. Heavy oil derived from the process is admixed with the powdered coal in approximately equal proportions by weight to form the paste. A hydrogenation catalyst, e. g., iron sulfate in an amount equivalent to about 1 per cent by weight, is incorporated in the paste. The paste is mixed with hydrogen, preheated to the operating temperatures, generally about 850° F., and passed into converters under a pressure of from about 4,000 to about 10,000 pounds per square inch. This step is called the liquid phase hydrogenation step of the process. Vapors are separated from the residual solids and liquid at the operating pressure and temperature. Unreacted hydrogen and most of the oil are removed as vapors. The vapors are cooled to condense the oil, and the hydrogen is recycled. Heavy oil is separated from the residual solids. The heavy oil is used for preparing the paste, while residual solids are used as fuel. The light oils are subjected to vapor phase hydrogenation for conversion to gasoline. In this step, oil vapors and hydrogen are passed over a catalyst, e. g., tungsten sulfide, at a pressure of about 4,500 pounds per square inch. Oils boiling above the motor fuel boiling range are recycled to the process.

An important element of cost in conventional coal liquefaction processes is in the preparation of the coal for hydrogenation. In the process of the present invention it is not necessary to pulverize the coal feed or to prepare a paste in conventional manner. Elimination of the pulverizing and conventional pasting steps results in a substantial saving in operating costs.

An object of this invention is to provide an improved process for the hydrogenation of coal.

Another object is to provide an improved process for the production of oil from coal by liquid phase reaction of coal with hydrogen.

Other objects and advantages will be apparent to those skilled in the art from the following detailed description of the invention.

In accordance with the process of this invention, coal is liquefied, the liquefied coal is atomized, and subjected to hydrogenation in a dispersed condition at an elevated temperature and pressure.

Coal may be rendered plastic by heating. The

plastic point varies with different coals. Generally coal becomes plastic or liquefies at a temperature within the range of from about 550 to about 700° F. When coal is heated in the presence of a mineral oil, the coal and oil become miscible and may be mixed to form a substantially homogeneous viscous liquid. Some hydrocarbon oils, especially hydroaromatics, such as tetralin, decalin, and heavy oils obtained by hydrogenation of coal, act as solvents and aid in the liquefaction of the coal. At temperatures above about 700° F., there is a condensation of free radicals or unsaturated compounds (generated by thermal decomposition of coal substance) into materials more stable than the original coal substances. At temperatures above about 825° F., the rate of precipitation of insoluble polymer may exceed the rate of liquefaction. The coal should be kept at a temperature as low as possible during liquefaction and subsequent handling in the liquid state to prevent excessive precipitation of the solid polymer. The optimum temperature for liquefaction is dependent upon the type and source of the coal and the length of time in which the coal must be kept in liquid state prior to hydrogenation and is best determined by trial for any given coal.

When the coal is liquefied with the oil with mechanical mixing, a substantially homogeneous liquid mixture may be obtained. Finely divided solid particles may be present in the mixture. This mixture may be atomized without further treatment. On the other hand, when the particles of coal are extracted with oil without agitation about 65 per cent by weight of the coal is taken into solution in the oil leaving a porous friable residue. The liquefied coal or extract obtained by this method is substantially free from ash. The undissolved portion of the coal is suitable for reaction, in situ, to produce carbon monoxide and hydrogen by reaction with steam or with a mixture of steam and oxygen. With either method of liquefaction the residual solids may be used for the generation of synthesis gases or for production of hydrogen for the process.

In accordance with preferred practice of this invention, coal and oil are admixed to form a liquid at a temperature within the range of about 550 to 850° F. and the resulting liquid is atomized into a hydrogenation reactor operated at a temperature within the range of from about 750 to about 850° F. and a pressure above about 1000 pounds per square inch gauge. Hydrogen is preferably used as a dispersing medium for atomization of the coal. The coal may be lique-

fed at a temperature of 550 to 700° F. and the resulting liquid heated to a temperature within the range of from about 750 to about 850° F. prior to hydrogenation.

The quantity of liquid admixed with the coal to form a liquid stream which may be atomized with conventional equipment may vary considerably depending upon the type of coal and oil used in the preparation step. Generally, a quantity of oil equivalent to about 50 per cent by weight based on the weight of the coal is sufficient to provide a fluid feed stream which may be atomized.

The particle size of the coal fed to the process is not of particular importance. The smaller particles are more quickly liquefied. The particles should be of such size that substantially complete liquefaction takes place in a reasonable period of time. Generally it is desirable to use particles ranging from about  $\frac{1}{2}$ -inch in average diameter to powder.

With the present process it is not necessary to resort to fine grinding or pulverization of the coal prior to preparation of the feed as in conventional hydrogenation processes. It is contemplated that in most applications of the process, the coal will be reduced only to a particle size such that the largest particles are dissolved prior to discharge of the liquid from the liquefaction vessel. Coal may be crushed mechanically to a particle size of  $\frac{1}{2}$ -inch to  $\frac{1}{4}$ -inch in average diameter with a relatively small expenditure of power. Further reduction in size becomes progressively more expensive, pulverization by mechanical means requiring large expenditures of power. The process of the present invention represents a considerable saving in power requirements for the preparation of the feed over conventional methods of preparation.

The atomized coal may be hydrogenated under conditions satisfactory for conventional liquid phase hydrogenation of coal. Liquid phase coal hydrogenation is a well-known procedure. In atomized form, the liquefied coal is more reactive than in conventional paste form, hence the time required to effect a given percentage of conversion is somewhat less than for conventional procedures. The pressure under which the coal is hydrogenated may range from 1,000 to 10,000 pounds per square inch gauge or higher, and the temperature from 600 to 900° F.

In a preferred embodiment, the liquefied coal is atomized and suspended in hydrogen. The suspension is introduced into a fluidized bed of residual solid material resulting from the coal hydrogenation reaction. The solid residual particles are entrained in the product stream and are separated from the oil in subsequent separation steps of conventional design. The residual solid material contains unreacted carbon as well as ash from the coal and may be used as fuel or reacted with steam or with steam and oxygen to produce a mixture of carbon monoxide and hydrogen. About 70 per cent by weight of the coal charged to the process may be converted to fluid products by hydrogenation, the hydrogen consumption generally ranging from about 1.5 to about 3 per cent by weight based on the weight of the dry coal.

The invention will be more readily understood from the following detailed description and the accompanying drawing.

The figure is a diagrammatic elevational view illustrating a preferred mode of carrying out the process of the present invention.

With reference to the drawing, coal of a suitable particle size is supplied to a hopper 5 through a conduit 6. From the hopper the coal may be fed through conduit 7 into liquefaction vessel 8 or through conduit 9 into liquefaction vessel 10. Any number of such vessels may be employed. With two vessels, as illustrated, one of the vessels is charged with coal and oil to prepare a liquefied coal feed stream for hydrogenation while the other is being discharged to the hydrogenation reactor. When a vessel has been filled with coal from the hopper, inert gas from line 12 may be admitted to the vessel to purge it of air. Valve 13, associated with vessel 8, and valve 14, associated with vessel 10, are provided for this purpose. Air and other gases may be vented from the vessels to line 15. Gases from vessel 8 are vented to line 15 through valve 16; those from vessel 10, through valve 17.

Preheated oil from line 18 may be admitted to vessel 8 through valve 19 and to vessel 10 through valve 20. When a vessel is filled with coal and oil the valves are closed and the coal particles at least partially liquefied due to the combined effect of heating and the solvent or plasticizing action of the hot oil. A substantially homogeneous liquid mixture of coal substance and oil is thus obtained.

Mechanical mixers, not illustrated in the drawing, may be supplied to insure complete disintegration of the coal, if desired.

As illustrated in the drawing; the coal is subjected to intimate contact with hot oil without agitation, effecting solution of a part of the coal in the oil and leaving a porous friable residue in the liquefaction vessels 8 and 10. The resulting liquid, comprising liquefied coal and oil, is discharged from vessel 8 through valve 23 and from vessel 10 through valve 24 to a charge pump 25 as feed for the hydrogenation step.

Inert gas from line 12 may be admitted to the vessel during the period of discharge to the feed pump. Gas from line 12 may be supplied under pressure to build up a pressure within the vessel and aid in the removal of liquid from the residual solid. This gas may be heated if desired to an elevated temperature. This porous friable residue remaining in the liquefaction vessel is in a state nearly ideal for gasification. A mixture of steam and oxygen may be supplied to the liquefaction of vessels through line 27. The flow of gas from line 27 is controlled by valves 28 and 29 associated with vessels 8 and 10, respectively. The resulting products of gasification may be discharged into line 15 for further use as desired.

Catalyst may be admitted through line 30 into admixture with the stream of liquefied coal and oil.

From the charge pump 25 the liquefied coal and oil stream is passed through a heating coil 32 and charged through line 33 into an atomizer 34 associated with a hydrogenation reactor 35. The coal feed stream may be fed directly from the charge pump 25 to the atomizer 34 through line 36 as controlled by valve 37. Since it is generally desirable to carry out the hydrogenation reaction at a pressure above about 1,000 pounds per square inch gauge and often not desirable to subject the heating coil 32 to excessive pressure, a second charge pump 38 may optionally be provided to increase the pressure of the hot charge stream immediately prior to introduction of the stream to the atomizer 34.

Hydrogen is admitted to the system through

line 40. Fresh and recycled hydrogen are pumped by a pump 41 through line 42 into the atomizer 34. In the atomizer 34, which may be of any conventional type, the liquefied coal feed stream is broken up into small droplets and dispersed in the stream of hydrogen from line 42. From the atomizer, the dispersion of liquefied coal and hydrogen is discharged directly into the hydrogenation zone 35. In the dispersed state, the hydrogenation reaction proceeds rather rapidly.

Somewhat more hydrogen is usually required for atomization and dispersion of the atomized coal stream than is required in the conventional liquid phase hydrogenation. This merely results in a higher recycle rate, since hydrogen consumption, for a given percentage conversion, is not appreciably affected.

The hydrogenation reaction results in precipitation of ash and the more difficultly hydrogenatable fraction of the coal substance as solids. These solids are entrained in the effluent stream discharged from the hydrogenation zone 35 through line 47. The hydrogenation effluent is passed to a separation system 48 wherein it is separated into various fractions. Any of several known conventional methods of separation may be employed. A gaseous fraction is recycled to the hydrogenation reactor through line 49 to pump 41. A portion of the gaseous fraction may be purged from the system through line 51. A light oil fraction is taken from the separation system through line 52 and a middle oil fraction through line 53 for further processing. In accordance with general conventional practice, the middle oil stream is subjected to further hydrogenation in vapor phase to produce motor fuels. Residual solids separated from the oils in the separation system 48 are discharged through line 54.

Heavy oil is discharged from the separation system through line 56 as a recycle stream to the liquefaction vessels 8 and 10. A portion of the heavy oil may be withdrawn for other uses through line 57. Other oils may be supplied if desired to the heavy oil recycle stream through line 58. The heavy oil stream is heated in a heating coil 60 to the desired temperature prior to admission to the liquefaction vessels 8 and 10 through line 18. All of the heat required for the process may be supplied by the hot oil stream.

It will be understood by those skilled in the art that various alternatives are available in the way of equipment and methods of handling the various streams and utilizing the heat contents to maximum advantage. In the interest of simplicity, various conventional pieces of apparatus such as control valves, heat exchangers, and the like, have been omitted.

In a typical operation of a process such as illustrated in the drawing, Pittsburgh Bed coal containing about 2 per cent water, 31 percent volatile matter, 58 per cent fixed carbon, and 9 per cent ash, as received, is subjected to hydrogenation. The coal is charged to a liquefaction vessel in the form of lumps about  $\frac{1}{2}$  to  $\frac{1}{4}$  inch in average diameter. This coal is mixed with heavy oil obtained from the hydrogenation of coal in an amount approximately equal in weight to the weight of the coal. The oil is preheated to a temperature of about 850° F. before admixture with the coal, resulting in a temperature of about 750° F. in the liquefaction vessel. About

65 per cent by weight of the coal is liquefied or extracted by the liquid oil without agitation, leaving a porous friable carbonaceous residue.

The resulting liquid comprising liquefied coal 5 is atomized with hydrogen into a reactor at about 750° F. and about 1,000 pounds per square inch gauge.

Obviously many modifications and variations of the invention as hereinabove set forth may be made without departing from the spirit and scope thereof and therefore only such limitations should be imposed as are indicated in the appended claims.

We claim:

1. A process for the hydrogenation of fusible coal which comprises contacting particles of said coal having an average diameter smaller than about  $\frac{1}{2}$  inch with a hydroaromatic oil at a temperature within the range of from about 550 to 20 about 850° F. and above the plastic point of said coal, mixing the coal and oil at said temperature for a period of time sufficient to form a substantially homogeneous liquid mixture, contacting said liquid mixture with hydrogen in a hydrogenation zone at a temperature within the range of from about 600 to about 900° F. and a pressure within the range of from about 1,000 to about 10,000 pounds per square inch gauge whereby hydrogenation of said liquid takes place with the 30 formation of particulate solid residue, maintaining a fluidized bed of said particulate solid residue within said hydrogenation zone, discharging resulting fluid products of hydrogenation and solid residue from said hydrogenation zone, and recovering said fluid products.
2. A process for the hydrogenation of fusible coal which comprises contacting particles of said coal having an average diameter within the range of from about  $\frac{1}{4}$  inch to about  $\frac{1}{2}$  inch with a 40 hydroaromatic oil at a temperature within the range of from about 550 to about 850° F. and above the plastic point of said coal, mixing the coal and oil at said temperature for a period of time sufficient to form a homogeneous liquid mixture, atomizing said liquid mixture, suspending the atomized liquid in hydrogen at a temperature within the range of from about 600 to 45 about 900° F. and a pressure within the range of from about 1,000 to about 10,000 pounds per square inch gauge whereby hydrogenation of said liquid takes place with the formation of particulate solid residue, introducing said suspension at said hydrogenation temperature and pressure into a fluidized bed of particulate residual solid material resulting from the hydrogenation reaction, 50 discharging the resulting fluid products of hydrogenation and solid residue from said hydrogenation zone, and recovering said fluid products.
3. A process for the hydrogenation of fusible coal which comprises contacting particles of said coal having an average diameter within the range of from about  $\frac{1}{4}$  inch to about  $\frac{1}{2}$  inch with a hydroaromatic oil at a temperature within the range of from about 550 to about 850° F. and above the plastic point of said coal, mixing the coal and oil at said temperature for a period of time sufficient to form a homogeneous liquid mixture, atomizing said liquid mixture, suspending the atomized liquid in hydrogen at a temperature within the range of from about 600 to about 900° F. and a pressure within the range of from about 1,000 to about 10,000 pounds per square inch gauge whereby hydrogenation of said liquid takes place with the formation of particulate solid residue, introducing said suspension at said hydrogenation temperature and pressure into a fluidized bed of particulate residual solid material resulting from the hydrogenation reaction, discharging the resulting fluid products of hydrogenation and solid residue from said hydrogenation zone, and recovering said fluid products.

ERNEST F. PEVERE.  
HOWARD V. HESS.  
GEORGE B. ARNOLD.

References Cited in the file of this patent

UNITED STATES PATENTS

| Number    | Name             | Date           |
|-----------|------------------|----------------|
| 1,864,496 | Pier et al.      | June 21, 1932  |
| 1,890,435 | Krauch et al.    | Dec. 6, 1932   |
| 2,215,190 | Pier et al.      | Sept. 17, 1940 |
| 2,436,938 | Scharmann et al. | Mar. 2, 1948   |
| 2,464,271 | Storch et al.    | Mar. 15, 1949  |
| 2,476,999 | Orchin           | July 26, 1949  |